

Patented Aug. 23, 1927.

1,640,315

# UNITED STATES PATENT OFFICE.

HORACE FREEMAN, OF SHAWINIGAN FALLS, QUEBEC, CANADA, ASSIGNOR OF ONE-HALF TO CANADA CARBIDE COMPANY, LIMITED, OF MONTREAL, CANADA.

## PROCESS OF MANUFACTURE OF ALKALI-METAL SULPHIDES.

No Drawing. Original application filed February 14, 1923, Serial No. 619,030. Divided and this application filed June 30, 1924. Serial No. 723,135.

This invention is a division from my former application, Serial No. 619,030, filed the 14th day of February, 1923, and relates to improvements in the manufacture of sodium sulphide, and the primary object is to obtain a higher yield of an improved product and in a less time than has heretofore been the case.

A further object is to overcome the inherent difficulties in dealing with sodium sulphide arising from its practically infusible nature.

A still further object is to render the electric furnace available for this manufacture.

The parent application relates broadly to the manufacture of sodium sulphide using other sulphides to produce with the sodium sulphide mixture of sulphides having relatively low melting points. The additional sulphides are identified as those soluble in aqueous solutions of sodium sulphide and particularly potassium sulphide. The present application relates to the use of those sulphides which are insoluble in concentrated aqueous solutions of sodium sulphide, and more particularly to the heavy metal sulphides and certain alkaline earth metal sulphides, namely, calcium and barium sulphides.

At present sodium sulphide is commercially produced by heating to a bright red heat in a fuel fired furnace, a mixture of sodium sulphate with a carbonaceous reducing agent, such as coal or sawdust.

As sodium sulphate is fusible, and sodium sulphide is not fusible at temperatures which are commercially practicable in this art, it is found that when the proportion of sulphate predominates, as during the earlier stages of the reduction, the charge remains liquid. When about fifty per cent of sulphide is formed, the mass thickens and becomes more solid; as a consequence the necessary contact between the reacting particles is prevented and the reduction is checked.

For this reason, the product of this method of operation seldom contains more than sixty-five per cent of sodium sulphide and is obtained from the furnace in the form of a

semi-solid mass, which is practically electrically non-conductive even when hot.

In carrying out this process I have found that the imperfections of this method of production, viz., the low grade of the fuel fired furnace product and the long period required for the reaction, are due to the infusibility of sodium sulphide, which also introduces complications in its removal from the furnace.

An object of this invention is to render the furnace charge fusible throughout the period of operation and in some instances at a lower temperature than is generally used for the reduction. The charge being fluid, the reaction is more complete and the yield of sodium sulphide is greater. Also, owing to its fluidity, the charge is electrically conductive enabling use of the electric furnace for heating in all stages and further enabling the sulphide to be tapped from the furnace.

I have found that sodium sulphide which, in the pure state, is infusible, or practically so, forms readily fusible compounds when mixed with other sulphides, such as those of potassium, calcium, barium, strontium, copper, zinc, lead, iron, and many others.

During the course of a long investigation of the products so obtained, I have found that the lowering of the fusing point of sodium sulphide is particularly great when potassium sulphide is added to it. Thus, a mixture in proportion of one mole of sodium sulphide to one mole of potassium sulphide melts to a thin, mobile liquid at 420° C., while the addition of only ten per cent of potassium sulphide to sodium sulphide produces a mixture melting at 570° C.

Furthermore, the double sulphides of sodium with lead, with zinc, with iron and with copper are very mobile liquids at temperatures much below 700° C. Also the double sulphides of sodium with the alkaline earth metals fuse readily at relatively low temperatures.

Of the alkaline earth metal sulphides, barium sulphide and calcium sulphide have an additional characteristic in common with the heavy metal sulphides, namely, they are

insoluble in concentrated aqueous solutions of sodium sulphide. In this connection it may be noted that iron and barium sulphides are to some extent soluble in very dilute 5 solutions of sodium sulphide.

In carrying out this process for the production of sodium sulphide the above described properties are made use of in the following manner according to the product 10 it is desired to obtain.

If the product required is hydrated sodium sulphide, free from admixture with other sulphides, the reduction of sodium sulphate is carried out with a reducing agent, such as 15 coal, in the ordinary manner, but when or before the previously mentioned thickening of the reacting mass takes place, a proportion of an insoluble sulphide is added sufficient to make the charge liquefy or to keep 20 the same liquid. A very small proportion of the added sulphide will liquefy the charge at a temperature of 1,000° C., while the addition of a molecular proportion of lead sulphide will cause liquefaction of the sodium 25 sulphide at 550° C., and when a molecular proportion of zinc sulphide is used, at 620° C.

The common sulphide ores are used for this purpose or refined or recovered sulphides may be used as obtained in the later 30 steps of the process.

The insoluble sulphide may be added to the charge of sulphate and its reducing agent prior to feeding them into the furnace, or it may be added at any subsequent stage in order to bring about the desired 35 result, viz., the maintaining of the sodium sulphide in the reaction mixture in a liquid condition so that reduction may proceed 40 to completion. As an alternative a metal sulphate may be added which will reduce to a sulphide to fuse with the sodium sulphide.

During the period of reduction the carbon 45 monoxide gas produced, easily and quietly escapes from the mobile liquid. When the evolution of gas ceases reduction is complete and the charge may be tapped or poured from the furnace.

The product of this operation is sodium 50 sulphide in admixture or combination with an insoluble sulphide. In order to obtain pure sodium sulphide from this material, it is necessary to lixiviate the mass with hot 55 water. The sodium sulphide is readily dissolved in the water but the other metal sulphide remains undissolved in the form of an extremely fine suspension, which, however, quickly settles on account of its 60 high specific gravity. The clear solution of sodium sulphide is therefore easily separated and allowed to crystallize; the product of crystallization being sodium sulphide free from other sulphides.

It is obvious that the fine sludge of the

added metal sulphide resulting from this operation is available after drying for re-use in the process of reduction.

If the sulphide product desired is that known as fused sodium sulphide and is to 70 be used without further refinement by crystallization, the presence of an insoluble metal sulphide would be objectionable. The presence of potassium sulphide or a soluble alkaline earth metal sulphide is ordinarily 75 not objectionable inasmuch as these sulphides will perform the same function as sodium sulphide in many of its various applications in the arts.

As previously stated, potassium sulphide 80 is particularly effective in rendering sodium sulphide fusible in the process of reduction. Less than ten per cent of the potassium sulphide is required and in most cases less than five per cent of the weight of sodium sulphide is a practicable proportion to use, although I do not desire to be confined to any particular proportion.

My process for producing the fused alkali metal sulphide consists in heating a mixture 90 of sodium sulphate with the desired proportion of potassium sulphate and a carbonaceous reducing agent. Potassium sulphide is formed coincidentally with sodium sulphide and the charge remains liquid while 95 the reduction is carried to completion. As an alternative I may add previously prepared potassium sulphide to the sodium sulphate charge undergoing reduction. The result is the same, i. e., the liquefaction of 100 the charge.

The process may be operated similarly using alkaline earth metal sulphides admixed with the sodium sulphate.

The product can then be tapped or run 105 from the furnace direct into containers for shipping, it may be cooled in moulds, or it may be quickly cooled on a rotating water-cooled drum and produced in the form of flakes as is now done with caustic soda and 110 with cyanide.

With the process here described the time required for reduction is much shortened and a smaller amount of the reducing agent is used than in the process heretofore practised. The reduction is carried much further than in the usual process, owing to the mobility of the charge in the furnace and the intimate contact of particles thereby 115 provided.

I do not desire to be confined to any particular form of furnace in carrying out this process, but I prefer and have used an electric furnace for the purpose, utilizing the charge itself as the resistor. The electric 125 furnace is preferred as it is more economical and avoids oxidation of the sulphide product, which is apt to take place in a fuel fired furnace. My process for the first time makes the electric furnace available for this 130

manufacture, allowing of the tapping of the liquid product and dispensing with the use of moving devices for stirring the charge.

- 5 In carrying out any of the variations of this process I may either add the desired sulphide or sulphides to the charge, or I may, as described, add the corresponding sulphate or sulphates which will be reduced 10 to sulphides coincident with the reduction of sodium sulphate. The product of the process here described contains larger percentages of available sulphide than is at all possible by the method now commonly used.

15 Having thus described my invention, what I claim is:—

1. The process of producing sodium sulphide which consists in heating sodium sulphate with a carbonaceous reducing agent 20 in the presence of a sulphide insoluble in concentrated aqueous solutions of sodium sulphide, whereby the sodium sulphide is maintained molten and freely fluid at a temperature under 1,500° C.

25 2. The process of producing sodium sulphide which consists in fusing sodium sulphate with a heavy metal sulphide in presence of a carbonaceous reducing agent, whereby the sodium sulphide produced by substantially complete reduction of the sulphate is capable of liquefaction.

3. The process of producing sodium sulphide, which consists in heating sodium sulphate with a carbonaceous reducing agent at 35 a temperature under 1,500° C. in the presence of a sulphide insoluble in concentrated aqueous solutions of sodium sulphide, lixiviating the sulphide product with water, separating the solution of sodium sulphide from the insoluble sulphide, and crystallizing the sodium sulphide from the solution.

4. The process of producing sodium sulphide, which consists in heating sodium sulphate with a carbonaceous reducing agent in 45 the presence of a heavy metal sulphide at such temperature that the formed sodium sulphide is maintained molten until after substantially complete reduction of the sodium sulphate is effected, lixiviating the sulphide product with water, separating the solution of sodium sulphide from the heavy metal sulphide, and crystallizing the sodium sulphide from the solution.

5. In a process for obtaining sodium sulphide, the procedure which consists in treating with water a solid mixture of sodium sulphide and a sulphide insoluble in concentrated aqueous solutions of sodium sulphide, dissolving the sodium sulphide, separating the solution from the insoluble sulphide and allowing sodium sulphide to crystallize from the solution.

6. In a process for obtaining sodium sulphide, the procedure which consists in treating with water a solid mixture of sodium

sulphide and a heavy metal sulphide, dissolving the sodium sulphide, separating the solution from the insoluble heavy metal sulphide and allowing sodium sulphide to crystallize from the solution.

7. The process of making sodium sulphide which comprises heating in an electric furnace sodium sulphate with a carbonaceous reducing agent and in presence of a sulphide of another metal insoluble in concentrated 75 aqueous solutions of sodium sulphide, by passing an electric current through the charge sufficient to maintain such temperature that the formed sodium sulphide is maintained molten and electrically conductive until after substantially complete reduction of the sodium sulphate is effected.

8. The process of making sodium sulphide which comprises heating sodium sulphate with a carbonaceous reducing agent 80 and in presence of a heavy metal sulphide in an electric furnace.

9. The product which comprises sodium sulphide fused with a sulphide of another metal which sulphide is insoluble in aqueous 90 solutions of sodium sulphide, the sodium sulphide content of the product being upwards of 50%.

10. A process for the substantially complete reduction of sodium sulphate to sodium sulphide, which consists in heating sodium sulphate and a heavy metal sulphide with a carbonaceous reducing agent at a temperature over 1,000° C.

11. A process for the substantially complete reduction of sodium sulphate to sodium sulphide, which consists in heating sodium sulphate and a metal sulphide insoluble in concentrated aqueous solutions of sodium sulphide with a carbonaceous reducing agent 100 at a temperature over 1,000° C.

12. A process for the substantially complete reduction of sodium sulphate to sodium sulphide, which comprises heating sodium sulphate with a carbonaceous reducing agent at a temperature sufficient for reduction and in presence of a heavy metal sulphide, whereby the sodium sulphide as it forms is fluxed and maintained molten until after substantially complete reduction of the sulphate.

13. A process for the substantially complete reduction of sodium sulphate to sodium sulphide, which comprises heating sodium sulphate with a carbonaceous reducing agent at a temperature sufficient for reduction and in presence of a metal sulphide insoluble in concentrated aqueous solutions of sodium sulphide, whereby the sodium sulphide as it forms is fluxed and maintained molten until after substantially complete reduction of the sulphate.

14. A process of making a sodium sulphide product with over 80% sodium sulphide content, which comprises fusing to-

gether sodium sulphate and a metal sulphide which is insoluble in concentrated aqueous solution of sodium sulphide, in presence of a carbonaceous reducing agent.

5 15. A process of making a sodium sulphide product of over 80% sodium sulphide content and free from sodium carbonate and sodium sulphate, which comprises reducing

sodium sulphate with a carbonaceous reducing agent at a temperature over 1,000° C. <sup>10</sup> and in presence of a metal sulphide which is insoluble in concentrated aqueous solutions of sodium sulphide.

In witness whereof, I have hereunto set my hand.

HORACE FREEMAN.